# EUROPEAN PATENT SPECIFICATION

(11) **EP 0 382 155 B1**
(45) Date of publication and mention of the grant of the patent: **11.08.1993**
(21) Application number: 90102275.6
(22) Date of filing: 06.02.1990
(51) Int. Cl.: C10M 169/04, C10M 111/02, C10M 173/02

(54) **Water soluble salt precoats for wire drawing**
Wasserlösliche Salzüberzüge zum Drahtziehen
Revêtements de sel soluble dans l'eau pour tréfiler

(30) Priority: 07.02.1989 US 307643
(43) Date of publication of application: 16.08.1990
(73) Proprietor: HENKEL CORPORATION (a Delaware corp.), Ambler, PA 19002 (US)
(72) Inventor: Tull, Thomas W., Southfield, Michigan 48076 (US)
(74) Representative: von Kreisler, Alek, Dipl.-Chem.

(56) References cited:
- GB-A- 2 003 923
- US-A- 2 957 825

## Description

This invention relates to modified water soluble salt precoats for use in the cold drawing of steel wire.

Water soluble salt coatings are often applied to steel wire in the form of aqueous solutions prior to drawing. The solution-coated wire is dried and the resulting salt coated wire is then drawn through conventional reducing dies using dry soap lubricants - a process well-known to this art. The water soluble salt coating acts as a lubricant carrier, pulling the dry soap box lubricant into the dies, thus providing lubrication. These dried-in-place, water soluble salt coatings have proven to be superior to other conventional coatings such as lime or borax coatings because of their improved ability to carry lubricant into the dies. A typical soluble salt composition used for the coating of steel (usually stainless steel) wire contains both sodium sulfate and borax. Such soluble salt compositions provide coatings with excellent crystalline structure, resulting in good soap lubricant pick-up when the coated wire is passed through a soap box, and therefore good drawability. However, such salt coating are prone to excessive moisture absorption upon exposure to ambient air, particularly when exposed to air having high humidity. Such moisture absorption seriously interferes with, or even prevents, the drawings of the coated wire. On the other hand, soluble salt coating which provide low moisture absorption provide little or no crystalline structure (i.e. amorphous or glaze type coatings) and are significantly inferior in both lubricant pick-up and drawability. This Hobson's choice problem has not previously been solved.

US-A-2 957 825 discloses a lubricant composition which comprises borax, sulphur salts and a soap. GB-A-2 003 923 discloses a metal working lubricant comprising a water soluble metallic soap such as sodium stearate in combination with alkali metal chlorides, sulphates and borates.

Compositions for coating steel wire have now been discovered which provide uniform coatings with good crystalline structure, soap pick-up, and drawability, while at the same time low moisture absorption even during humid days, i.e. low hygroscopicity.

The compositions of the invention, which are in the form of dry mixtures prior to dilution with water for use, in contain the following components:
A. from 50 to 99.99, preferably from 70 to 89.9% by weight K₂SO₄;
B. from 0 to 49.99, preferably from 10 to 29.9% by weight K₂B₄O₇ and/or KBO₂; and
C. from 0.01 to 5, preferably from 0.1 to 1.0% weight of an ammonium or potassium soap,

wherein up to 50% by weight, and preferably no more than 10% by weight, of the total potassium ions and ammonium ions present in A., B. and C. can be replaced with sodium ions. More preferably, substantially none of the potassium and ammonium are replaced with sodium ions, since the more sodium ions present, the greater the hygroscopicity. When sodium ions are present, they can be present in one or more of components A., B. and C., e.g. component C. can be partially or entirely a sodium soap. Also, component A. and/or B. can be a sodium or a potassium salt, or a mixture of such salts, provided the limitation on total quantity of sodium ion is maintained.

The fact that the above compositions provide good crystallinity on steel wire is completely unexpected, since the above compositions without component C. give non-uniform coatings on steel wire which are not useful as such since both soap pick-up and drawability are unsatisfactory. In some unknown manner, the presence of the soap provides an at least partially crystalline uniform coating when the composition in aqueous solution is applied to the steel wire which is then dried or allowed to dry.

The K₂SO₄ used as component A. can be chemically pure or of a technical grade; the latter being preferred due to cost considerations.

The K₂B₄O₇ used as component B. can also be chemically pure or a technical grade, and is generally available and used herein as the tetrahydrate (K₂B₄O₇·4H₂O). Similarly, the KBO₂, which can be used alone as component B, or in a mixture with K₂B₄O₇ in any proportions, can be chemically pure or a technical grade.

The ammonium or potassium soap is one or more ammonium and/or potassium salts of a C₁₂-C₂₂ fatty acid or mixture of two or more such C₁₂-C₂₂ fatty acids. The fatty acids are generally saturated and unbranched, with ammonium or potassium stearate being preferred for use herein, although mono- or di-olefinically unsaturated C₁₂-C₂₂ fatty acids can also be employed, either alone or in mixtures with each other and/or with saturated fatty acids. For example, ammonium and potassium soaps derived from the fatty acid mixtures obtained by the saponification of tallow oil or coconut oil, or a mixture thereof, can advantageously be employed as component C. Also, ammonium or potassium salts of branched or cycloaliphatic-containing C₁₂-C₂₂ fatty acids can also be employed herein, either alone or in mixtures with unbranched fatty acid salts. Also, ammonium or potassium rosin acids, e.g. abietic acid, can also be employed as component C.

The wires coated with the coating compositions of the invention are generally steel wires, and usually stainless steel wires. However, other wire substrates can also be coated with the present coating compositions such as mild steel, titanium, vanadium, tungsten, aluminum, copper, nickel, zirconium, etc., and alloys thereof.

The coatings are applied by contacting the wires with an aqueous solution of the composition of the invention, and allowing the resulting wet coating to dry in place, either with or without the application of heat. The aqueous solutions generally contain from 75 to 400 g/l of the composition in water, preferably from 150 to 250 g/l.

The wire is contacted with the solution by any convenient technique, either batch or a continuous strand, and allowing the resulting wet-coated wire to air dry before coiling for storage, shipping, or use. The coated wire is then passed through conventional cold reduction equipment using a soap box (e.g. containing a conventional dry soap lubricant). The coating on the wire functions as a carrier to carry the dry soap lubricant into the die.

The steps employed in the treatment of wire according to the invention include the following:
1. Cleaning the wire - cleaning compositions are well-known in the art and do not comprise part of the present invention.
2. Rinsing with water.
3. Pickling - here also, pickling compositions are well-known and the selection of a pickling composition is not part of the invention.
4. Rinsing with water.
5. Applying the coating composition of the invention as described above.
6. Drying the wire as described above to produce the coated wire of the invention.

The coated wire can then be drawn, also as described above.

The water used in preparing the aqueous solutions of the invention is preferably distilled or deionized water, but tap water can also be used provided it is not overly hard and has a low dissolved sodium salts content.

The invention will be illustrated but not limited by the following examples.

### EXAMPLES

### EXAMPLE 1

The following aqueous compositions were tested for their morphology and hygroscopicity, when coated on stainless steel panels. Stainless steel panels were coated with each of the following compositions by immersing the panels in the aqueous composition, removing the panels from the aqueous composition, and allowing them to flash (air) dry.
a) 187.2 g of a mixture of 75 wgt % Na₂SO₄ and 25 wgt % sodium tetraborate·10H₂O per liter of deionized water.
   Use temperature 88°C (190°F).
b) 187.2 g of mixture of 75 wgt % K₂SO₄ and 25 wgt % K₂B₄O₇·4H₂O per liter of dionized water.
   Use temperature 88°c (190°F).
c) to an aqueous solution prepared as in a) was added 5 g/l of sodium stearate.
   Use temperature 88°C (190°F).
d) to an aqueous solution prepared as in b) was added 5 g/l of ammonium stearate.
   Use temperature 88°C (190°F).

The sections of stainless steel panel coated with the above compositions were then tested for hygroscopicity and morphology. The test results are set forth in Table I below. In Table I, RH = relative humidity.

As can be seen from Table I, the composition of the invention, composition d), produced a coating with good crystallinity, and low hygroscopicity.

### EXAMPLE 2

This example shows the effect of relative ratios of sodium and potassium ions on the hygroscopicity of the water soluble salt coatings. In this example, stainless steel panels were coated in accordance with Example 1 using the following compositions, at a concentration of 187.2 g/l in deionized water, set forth in Table II below together with test results. In Table II, M = molarity or gm-moles/liter of solution and RH = relative humidity.

### EXAMPLE 3

This example shows the relative hygroscopicity of lime coatings compared to the coating from a known sodium based salt composition and a low sodium salt composition of the invention. The coatings were produced on samples of the stainless steel wire used in Example 1 according to the procedure of Example 1 from the following aqueous compositions:
j) 187.2 g of mixture of 75 wgt % Na₂SO₄ and 25 wgt % sodium tetraborate·10H₂O per liter of dionized water.
   Use temperature 88°C (190°F).
k) 187.2 g of a mixture of 79 wgt % K₂SO₄, 20 wgt % sodium tetraborate·10H₂O, and 1 mole % of ammonium stearate per liter of deionized water.
   Use temperature 88°C (190°F).
l) 3% by weight of lime in deionized water.
   Use temperature 88°C (190°F).
m) 6% by weight of lime in deionized water.
   Use temperature 88°C (190°F).

The results are shown in Table III below.

As can be seen from Table III above, composition k) in accordance with the invention has significantly reduced hygroscopicity compared to lime coatings l) and m).

### EXAMPLE 4

Ten difference coating bath compositions were evaluated for moisture pick up, morphology, coating uniformity, and crsytals per inch on stainless steel panels.

The stainless steel panels were coated with the coating compositions and coating baths set forth in Table IV, according to the process given in Example 1, except that the wet-coated panels were dried using a 10 minute bake at 250°F. Moisture pick-up was determined in a chamber which allowed constant temperature and humidity of 80°F and 92% respectively. A Surtronic 3 surface prophylometer was used to determine the number of crystals per inch of caoting. Coating characterization and coating appearance were determined by visual observation.

In Table IV, coating compositions F, G, and J are compositions in accordance with the invention, while compositions A, B, C, D, E, H and I are comparison compositions. As can be seen from Table IV, compositions F, G, and J produced uniform coatings while exhibiting low moisture pick up. The only comparison composition that produced a uniform coating was composition B, which however exhibited an unacceptably high moisture pick up. In fact, compositions A, B and C all exhibited unacceptably high moisture pick up, and hence poor wire drawability properties in humid conditions. Coating composition E contains potassium sulfate and sodium stearate soap in accordance with the compositions of the invention, except that the sodium stearate soap is present in too high a quantity, resulting in a non-uniform, mostly glaze coating, having unacceptable wire drawing properties. Coating compositions D, H, and I which are potassium salt compositions in accordance with the invention except that no soap is present therein, all produced unacceptable non-uniform coatings and hence unacceptability inconsistent wire drawing characteristics. In comparing coating compositions F, G and J of the invention, composition J containing an alkali metal tetraborate produced the most crystalline coating. Hence, the presence of a tetraborate in the coating compositions of the invention, while optional, is nonetheless highly preferred.

## Claims

1. A composition for coating steel wire to facilitate the cold drawing thereof, said composition comprising:
(A) from 50 to 99.99 % by weight of a component selected from the group consisting of Na₂SO₄, K₂SO₄, and mixtures thereof;
(B) from 0 to 49.99 % by weight of a component selected from the group consisting of Na₂B₄O₇, NaBO₂, K₂B₄O₇, KBO₂ and mixtures of any two or more thereof; and
(C) from 0.01 to 5 % by weight of a component selected from the group consisting of potassium soaps, sodium soaps, and ammonium soaps;
wherein the percentages by weight are based on the total weight of components A, B, and C in the composition, and wherein not more than 50 % by weight of the total of sodium plus potassium plus ammonium ions in components A, B, and C of the composition consists of sodium ions.

2. A composition according to claim 1, wherein component C is selected from the group consisting of ammonium stearate, potassium stearate, and sodium stearate.

3. A composition according to claim 1 wherein not more than 10 % by weight of the total of sodium plus potassium plus ammonium ions in the composition consists of sodium ions.

4. A composition according to claim 1, wherein substantially none of the ions in the composition are sodium ions.

5. A composition according to claim 1, wherein component A is present in from 70 to 89.9 % by weight.

6. A composition according to claim 1, wherein component B is present in from 10 to 29.9 % by weight.

7. A composition according to claim 1, wherein component C is present in from 0.1 to 1.0 % by weight.

8. A composition according to claim 1, wherein component B is selected from K₂B₄O₇ and Na₂B₄O₇.

9. A composition according to claim 1, wherein the composition includes water which dissolves components A, B, and C to form an aqueous solution.

10. A composition according to claim 9, wherein the composition contains from 70 to 400 grams of the total of components A, B, and C per liter of solution.

11. A composition according to claim 10, wherein the aqueous solution contains from 150 to 250 grams of the total of components A, B, and C per liter of solution.

12. A method for the drawing of steel wire, the improvement comprising coating the wire prior to drawing with a composition comprising:
(A) from 50 to 99.99 % by weight of a component selected from the group consisting of K₂SO₄, Na₂SO₄, and mixtures thereof;
(B) from 0 to 49.99 % by weight of a component selected from the group consisting of Na₂B₄O₇, NaBO₂, K₂B₄O₇, KBO₂, and mixtures of any two or more thereof; and
(C) from 0.01 to 5 % of a component selected from the group consisting of ammonium soaps, potassium soaps, sodium soaps, and mixtures of any two or more thereof;
wherein the percentages by weight are based on the total weight of components A, B, and C in said composition, and wherein not more than 50 % by weight of the total of sodium plus potassium plus ammonium ions in the composition consists of sodium ions.

13. The method of claim 12 wherein the steel wire is stainless steel.

14. A method according to claim 12 wherein, component C is selected from the group consisting of ammonium stearate, potassium stearate, and sodium stearate.

15. A method according to claim 12 wherein not more than 10 % by weight of the total of sodium plus potassium plus ammonium ions in the composition consists of sodium ions.

16. A method according to claim 12, wherein substantially none of the ions in the composition are sodium ions.

17. A method according to claim 12, wherein component A is present in from 70 to 89.9 % by weight.

18. A method according to claim 12 or 17, wherein component B is present in from 10 to 29.9 % by weight.

19. A method according to claim 12 or 18, wherein component C is present in from 0.1 to 1.0 % by weight.

20. A method according to claim 12, wherein component B is selected from K₂B₄O₇ and Na₂B₄O₇.

21. A method according to claims 12 to 20, wherein the composition includes water which dissolves components A, B, and C to form an aqueous solution.

22. A method according to claims 21, wherein the composition contains from 70 to 400 grams of the total of components A, B, and C per liter of solution.

23. A method according to claims 22, wherein the aqueous solution contains from 150 to 250 grams of the total of components A, B, and C per liter of solution.

## Patentansprüche

1. Zusammensetzung zur Beschichtung von Stahldraht zur Erleichterung des Kaltziehens desselben, umfassend
(A) 50 bis 99,99 Gew.-% einer Komponente, die aus der aus Na₂SO₄, K₂SO₄ und deren Gemischen bestehenden Gruppe ausgewählt ist;
(B) 0 bis 49,99 Gew.-% einer Komponente, die aus der aus Na₂B₄O₇, NaBO₂, K₂B₄O₇, KBO₂ und Gemischen aus zweien oder mehreren dieser Verbindungen bestehenden Gruppe ausgewählt ist;
(C) 0,01 bis 5 Gew.-% einer Komponente, die aus der aus Kaliumseifen, Natriumseifen und Ammoniumseifen bestehenden Gruppe ausgewählt ist;
wobei die Gew.-%-Angaben auf das Gesamt-Gewicht der Komponenten A, B und C in der Zusammensetzung bezogen sind und worin nicht mehr als 50 Gew.-% der Gesamt-Menge aus Natrium- plus Kalium- plus Ammonium-Ionen in den Komponenten A, B und C der Zusammensetzung aus Natrium-Ionen bestehen.

2. Zusammensetzung nach Anspruch 1, worin die Komponente C aus der aus Ammoniumstearat, Kaliumstearat und Natriumstearat bestehenden Gruppe ausgewählt ist.

3. Zusammensetzung nach Anspruch 1, worin nicht mehr als 10 Gew.-% der Gesamt-Menge aus Natrium- plus Kaliumplus Ammonium-Ionen in der Zusammensetzung aus Natrium-Ionen bestehen.

4. Zusammensetzung nach Anspruch 1, worin im wesentlichen keine Ionen in der Zusammensetzung Natriuum-Ionen sind.

5. Zusammensetzung nach Anspruch 1, worin die Komponente A in einer Menge von 70 bis 89,9 Gew.-% vorliegt.

6. Zusammensetzung nach Anspruch 1, worin die Komponente B in einer Menge von 10 bis 29,9 Gew.-% vorliegt.

7. Zusammensetzung nach Anspruch 1, worin die Komponente C in einer Menge von 0,1 bis 1,0 Gew.-% vorliegt.

8. Zusammensetzung nach Anspruch 1, worin die Komponente B aus K₂B₄O₇ und Na₂B₄O₇ ausgewählt ist.

9. Zusammensetzung nach Anspruch 1, worin die Zusammensetzung Wasser enthält, das die Komponenten A, B und C unter Bildung einer wäßrigen Lösung auflöst.

10. Zusammensetzung nach Anspruch 9, worin die Zusammensetzung 70 bis 400 g der Gesamt-Menge der Komponenten A, B und C pro 1 Liter Lösung enthält.

11. Zusammensetzung nach Anspruch 10, worin die Zusammensetzung 150 bis 250 g der Gesamt-Menge der Komponenten A, B und C pro 1 Liter Lösung enthält.

12. Verfahren zum Ziehen von Stahldraht, worin die Verbesserung das Beschichten des Drahtes vor dem Ziehen mit einer Beschichtung umfaßt, die
(A) 50 bis 99,99 Gew.-% einer Komponente, die aus der aus Na₂SO₄, K₂SO₄ und deren Gemischen bestehenden Gruppe ausgewählt ist;
(B) 0 bis 49,99 Gew.-% einer Komponente, die aus der aus Na₂B₄O₇, NaBO₂, K₂B₄O₇, KBO₂ und Gemischen aus zweien oder mehreren dieser Verbindungen bestehenden Gruppe ausgewählt ist;
(C) 0,01 bis 5 Gew.-% einer Komponente, die aus der aus Kaliumseifen, Natriumseifen und Ammoniumseifen bestehenden Gruppe ausgewählt ist;
umfaßt, wobei die Gew.-%-Angaben auf das Gesamt-Gewicht der Komponenten A, B und C in der Zusammensetzung bezogen sind und worin nicht mehr als 50 Gew.-% der Gesamt-Menge aus Natrium- plus Kalium- plus Ammonium-Ionen in den Komponenten A, B und C der Zusammensetzung aus Natrium-Ionen bestehen.

13. Verfahren nach Anspruch 12, worin der Stahldraht aus nichtrostendem Stahl ist.

14. Verfahren nach Anspruch 12, worin die Komponente C aus der aus Ammoniumstearat, Kaliumstearat und Natriumstearat bestehenden Gruppe ausgewählt ist.

15. Verfahren nach Anspruch 12, worin nicht mehr als 10 Gew.-% der Gesamt-Menge aus Natrium- plus Kaliumplus Ammonium-Ionen in der Zusammensetzung aus Natrium-Ionen bestehen.

16. Verfahren nach Anspruch 12, worin im wesentlichen keine Ionen in der Zusammensetzung Natrium-Ionen sind.

17. Verfahren nach Anspruch 12, worin die Komponente A in einer Menge von 70 bis 89,9 Gew.-% vorliegt.

18. Verfahren nach Anspruch 12 oder 17, worin die Komponente B in einer Menge von 10 bis 29,9 Gew.-% vorliegt.

19. Verfahren nach Anspruch 12 oder 18, worin die Komponente C in einer Menge von 0,1 bis 1,0 Gew.-% vorliegt.

20. Verfahren nach Anspruch 12, worin die Komponente B aus K₂B₄O₇ und Na₂B₄O₇ ausgewählt ist.

21. Verfahren nach den Ansprüchen 12 bis 20, worin die Zusammensetzung Wasser enthält, das die Komponenten A, B und C unter Bildung einer wäßrigen Lösung auflöst.

22. Verfahren nach Anspruch 21, worin die Zusammensetzung 70 bis 400 g der Gesamt-Menge der Komponenten A, B und C pro 1 Liter Lösung enthält.

23. Verfahren nach Anspruch 22, worin die Zusammensetzung 150 bis 250 g der Gesamt-Menge der Komponenten A, B und C pro 1 Liter Lösung enthält.

## Revendications

1. Une composition pour le revêtement d'un fil d'acier pour en faciliter le tréfilage, ladite composition comprenant :
(A) de 50 à 99,99 % en poids d'un composant choisi dans le groupe constitué de Na₂SO₄, K₂SO₄ et leurs melanges ;
(B) de 0 à 49,99 % en poids d'un composant choisi dans le groupe constitué de Na₂B₄O₇, NaBO₂, K₂B₄O₇, KBO₂ et des mélanges quelconques de deux ou de plusieurs d'entre eux ; et
(C) de 0,01 à 5 % en poids d'un composant choisi dans le groupe constitué par les savons de potassium, les savons de sodium et les savons d'ammonium ;
dans laquelle les pourcentages en poids sont rapportés au poids total des composants A, B et C dans la composition et dans laquelle pas plus de 50 % en poids du total des ions sodium plus potassium plus ammonium dans les composants A, B et C de la composition sont constitués d'ions sodium.

2. Une composition selon la revendication 1, dans laquelle le composant C est choisi dans le groupe constitué du stéarate d'ammonium, du stéarate de potassium et du stéarate de sodium.

3. Une composition selon la revendication 1, dans laquelle pas plus de 10 % en poids du total des ions sodium plus potassium plus ammonium, dans la composition, sont constitués d'ions sodium.

4. Une composition selon la revendication 1, dans laquelle pratiquement aucun des ions de la composition n'est un ion sodium.

5. Une composition selon la revendication 1, dans laquelle le composant A est présent en une proportion de 70 à 89,9 % en poids.

6. Une composition selon la revendication 1, dans laquelle le composant B est présent en une proportion de 10 à 29,9 % en poids.

7. Une composition selon la revendication 1, dans laquelle le composant C est présent en une proportion de 0,1 à 1,0 % en poids.

8. Une composition selon la revendication 1, dans laquelle le composant B est choisi parmi K₂B₄O₇ et Na₂B₄O₇.

9. Une composition selon la revendication 1, laquelle composition comprend de l'eau qui dissout les composants A, B et C pour former une solution aqueuse.

10. Une composition selon la revendication 9, laquelle composition contient de 70 à 400 g de composants A, B et C totaux par litre de solution.

11. Une composition selon la revendication 10, dans laquelle la solution aqueuse contient de 150 à 250 g des composants A, B et C totaux par litre de solution.

12. Un procédé pour le tréfilage d'un fil d'acier, comprenant le perfectionnement qui consiste à revêtir le fil avant le tréfilage avec une composition comprenant :
(A) de 50 à 99,99 % en-poids d'un composant choisi dans le groupe constitué de K₂SO₄, Na₂SO₄ et leurs mélanges ;
(B) de 0 à 49,99 % en poids d'un composant choisi dans le groupe constitué de Na₂B₄O₇, NaBO₂, K₂B₄O₇, KBO₂ et des mélanges quelconques de deux ou de plusieurs d'entre eux ; et
(C) de 0,01 à 5 % d'un composant choisi dans le groupe constitué par les savons d'ammonium, les savons de potassium et les savons de sodium ;
dans laquelle les pourcentages en poids sont rapportés au poids total des composants A, B et C dans ladite composition et dans laquelle pas plus de 50 % en poids du total des ions sodium plus potassium plus ammonium dans la composition sont constitués d'ions sodium.

13. Le procédé de la revendication 12, dans lequel le fil d'acier est un fil d'acier inoxydable.

14. Le procédé de la revendication 12, dans lequel le composant C est choisi dans le groupe constitué du stéarate d'ammonium, du stéarate de potassium et du stéarate de sodium.

15. Un procédé selon la revendication 12, dans lequel pas plus de 10 % du poids du total des ions sodium plus potassium plus ammonium, dans la composition, sont constitués d'ions sodium.

16. Un procédé selon la revendication 12, dans lequel pratiquement aucun des ions de la composition n'est un ion sodium.

17. Un procédé selon la revendication 12, dans lequel le composant A est présent en une proportion de 70 à 89,9 % en poids.

18. Un procédé selon la revendication 12 ou 17, dans lequelle composant B est présent en une proportion de 10 à 29,9 % en poids.

19. Un procédé selon la revendication 12 ou 18, dans lequel le composant C est présent en une proportion de 0,1 à 1,0 % en poids.

20. Un procédé selon la revendication 12, dans lequel le composant B est choisi parmi K₂B₄O₇ et Na₂B₄O₇.

21. Un procédé selon les revendications 12 à 20, dans lequel la composition comprend de l'eau qui dissout les composants A, B et C pour former une solution aqueuse.

22. Un procédé selon la revendication 21, dans lequel la composition contient de 70 à 400 g de composants A, B et C totaux par litre de solution.

23. Un procédé selon la revendication 22, dans lequel la solution aqueuse contient de 150 à 250 g des composants A, B et C totaux par litre de solution.
